

Jan. 13, 1953

R. D. PIKE ET AL

2,625,384

MINING OPERATION

Filed July 1, 1949



Fig. 1



Fig. 2

INVENTORS

ROBERT D. PIKE

BY MAX Y. SEATON

*Hammond, Miller*  
ATTORNEYS

## UNITED STATES PATENT OFFICE

2,625,384

## MINING OPERATION

Robert D. Pike and Max Y. Seaton, Greenwich, Conn., assignors to Food Machinery and Chemical Corporation, New York, N. Y., a corporation of Delaware

Application July 1, 1949, Serial No. 102,599

6 Claims. (Cl. 262—3)

1

This invention relates to a novel and economical method for mining trona. There has recently been discovered near Green River, Wyoming, a mineral deposit which is an almost level bed of trona which is about 95% water soluble, yielding a solution of sodium sesquicarbonate which is almost chemically pure, except for a small amount of coloring matter which may be removed by adsorption. The bed ranges from 10-15 feet thick and lies at a depth of approximately 1500 feet below the surface. This invention is applicable to the mining and recovery of trona and other soluble salts from this and similar salt beds.

No body of almost pure trona has hitherto been discovered. This mineral, while fairly common in arid regions, as hitherto known, is contaminated with considerable amounts of NaCl and Na<sub>2</sub>SO<sub>4</sub>. But in the Green River trona, NaCl is present only to the extent of about 0.1%, and Na<sub>2</sub>SO<sub>4</sub> occurs in even smaller percentage. Nor has any deposit of subterranean trona hitherto been discovered, all known deposits being on or very near the surface. The discovery, therefore, near Green River, Wyoming, of a vast body of almost pure subterranean trona of mineable thickness, is a unique occurrence presenting unusual problems in the mining and recovery thereof.

The roof conditions over this deposit are suitable for mining by the conventional room-and-pillar system which we propose to use for dry mining. In this method the trona is mined from so-called unit panels, which when mined out, contain numerous supporting pillars of the trona, outlining the rooms from which the ore has been removed from each side of the central access and haulageways, which are employed while the panels are being mined. The room pillars which are left in the panels, support the roof and the so-called barrier pillars separate the panels from each other and from the surrounding trona bed.

In following our method, we proceed with dry mining alone until a number of mined out panels are left which are sufficiently remote from the current dry mining operation to enable us to carry out solution mining without encountering the danger of flooding the dry mining workings. This may take a number of years, say three to five, depending upon the rate of production by dry mining. At the expiration of this time, in accordance with our invention, we start solution mining of the material in the room pillars and barrier pillars.

We may proceed to thus mine one panel, or preferably a pair of panels, one on each side of

the main access and haulageways, which were used in dry mining. We do this by laying a water pipe along the bottom surface level of the panel haulageway to discharge water at approximately ground temperature and about two-thirds of the way back towards the rear barrier pillar. Where the pipe enters the panel, we erect a bulkhead or retaining wall across the accessway, through which wall the pipe enters at its bottom level and also a drainage pipe is placed at the same level. This drainage pipe is used to lead the liquor from solution mining to the sump of a pump. We preferably extend this bulkhead to, or nearly to, the roof. If desired the walls adjacent the bulkhead may be lined with an insoluble material, such as concrete, for a suitable distance inward from the bulkhead to assure that the walls adjacent the bulkhead will not be attacked by the solution.

20 The supply pipe, or the two pipes, if a pair of mined out panels is to be treated at the same time, extends to the surface where it receives the water required for solution. This water entering the panel at a controlled rate of flow, first attacks 15 and dissolves the bottom of the room pillars in the immediate vicinity of the end of the pipe. This will eventually cause these pillars to collapse and as they become dissolved, the area of unsaturated solution spreads and dissolves more pillars, 25 thus eventually causing most of the roof to collapse and most of the pillars to go into solution.

20 All of the water introduced through the pipe from the surface necessarily eventually flows out through the drain pipe in the bottom of the bulkhead as a substantially saturated solution at the ground temperature. This solution flows to the suction of a pump, which we preferably install 35 nearby in the main haulage and accessway and this lifts the saturated solution to the surface.

40 As the solution flowing to the pump is always substantially saturated, the material in the immediate vicinity of the bulkhead and the pump, although soluble in water, is not attacked by the saturated solution. Of course, if the flow of 45 water were kept up long enough, all of the soluble material near the bulkhead and pump would eventually be dissolved and the barrier pillar between the panel and the main accessways, would be at least partially dissolved. We prefer to stop the flow of water considerably short of this, but, if necessary, all undesired solution of trona near the bulkhead and pump pit can be prevented by lining the walls at these points with an insoluble material.

50 Once having started solution mining, we pre-

fer to carry it on in step relation with the dry mining operation. We thus prefer to bring to the surface each day sufficient sodium carbonate by solution mining, so that when this has been recovered, the total production formerly had by dry mining alone, will remain unchanged.

The principal object of our invention is to set up mining conditions in the trona whereby a considerable percentage of the total tonnage of  $\text{Na}_2\text{CO}_3$  produced is from low cost solution mining of the mined out panels.

A further object of our invention is to combine the production of sodium carbonate by solution mining and dry mining. This we prefer to do by heating the solution pumped up from the solution mining operations, and dissolving dry mined trona in it. The combined solution may then be clarified and used for the production of sodium carbonate by any suitable method, as for example, running to dryness in a rotary kiln, or drying in ponds on the surface by solar evaporation. An advantage of this latter method resides in its ability to crystallize out pure sodium carbonates, leaving what  $\text{NaCl}$  and  $\text{Na}_2\text{SO}_4$  may have been picked up in the solution mining operation, in the remaining mother liquor, which is then discarded.

Having described our invention in general terms, we now refer to the drawings of which—

Figure 1 shows a diagrammatic layout of a plan for underground mining, embodying our invention; and

Figure 2 shows a longitudinal section through a panel along the accessway in which the pipe is laid.

In the drawings, 10 is an operating shaft which may be either inclined or vertical, designed to receive mined trona and to raise the same and deposit it on the surface. At 11 is indicated an escape and air circulation shaft, which with slight modification may be used for full operation. The main entries for access, haulage and air circulation are shown at 12, 13, 14, 15 and 16. A typical mined out panel is shown at 17 and its companion panel in which dry mining is progressing, is shown at 18, although the precise location of 18 is open to considerable choice. While a generally rectangular dry mining operation has been shown, it will be understood that radial operation of mining shafts from a central access shaft and other arrangements may be used.

Panel 19, together with 17, may be considered as typical panels for solution mining. The room pillars are of various forms, but two types are indicated as 22, 23, the latter appearing in both Figures 1 and 2. The so-called barrier pillars are indicated at 24, 25 and 26. The pipe 28 may be laid in accessway 27. The pump sump is indicated at 29 and the pump at 30.

In practice, we supply water in controlled amount from the surface through pipe 28 and we may not open the pump valve 31 until the water has accumulated to a depth corresponding to the top of the bulkhead 32. At this point, or sooner if desired, we open valve 31 and pump the solution to the surface. We prefer to continue to add water until attack begins on the barrier pillar 26. At this point we may shut off the water from the surface, but continue to pump solution to the surface until substantially all of it has been pumped out of the panel. By this time most of the roof of the panel will have collapsed, opening up drainage of solution containing both  $\text{Na}_2\text{CO}_3$  and  $\text{NaHCO}_3$  and  $\text{NaCl}$  from overlying structures,

but we have observed that these structures are so dense that they do not provide a sufficient flow of brine to be an important factor. In fact, the continuing stream produced by them from an entire mine will only amount to a few gallons per minute and can easily be dealt with.

We have found that it is desirable to supply water to the underground pipe at no lower temperature than the underground temperature of about 70° F., but during the winter months the water available on the surface is at a considerably lower temperature and should be heated to the ground temperature before being introduced. This is because cold water will dissolve the trona more slowly and less than water at a higher temperature and also if the temperature of the water be below about 70° F., there is a tendency to decompose the trona dissolving  $\text{Na}_2\text{CO}_3$  preferentially and leaving solid  $\text{NaHCO}_3$  behind in the mine. But at temperatures at about 70° F. and above, the tendency is to dissolve trona without decomposition until the solution is saturated when an exchange will begin whereby  $\text{Na}_2\text{CO}_3$  goes into solution and  $\text{NaHCO}_3$  comes out until the trona sodium bicarbonate invariant point is reached, at which point solid trona is in equilibrium with solution. Thus at temperatures below 70° F., trona will be decomposed with preferential solutions of  $\text{Na}_2\text{CO}_3$  leaving  $\text{NaHCO}_3$  behind as a solid but at temperatures of 70° F. and above, there will be more of a tendency for trona to be dissolved as a whole, that is, congruently, although the possibility of selective solution of  $\text{Na}_2\text{CO}_3$  cannot be dismissed because of the large surface of the pillars and the long time of resistance of the water in the panel. Nevertheless, we have found that the more usual condition is solution of trona as such, that is, congruently, under the existing conditions, but our process deals with either condition, that is, congruent solution which leaves no solid sodium bicarbonate in the mine and solution which corresponds to the trona sodium bicarbonate invariant point which necessarily leaves a considerable amount of sodium bicarbonate in the mine. Intermediate conditions will often exist between these two extremes.

In citing an example for purpose of illustration, we shall assume that solution of the trona is congruent and that the temperature is 70° F.

In this example, it is assumed that an annual production of 500,000 tons equivalent  $\text{Na}_2\text{CO}_3$  is desired. Principal significant data for such production are given in the following:

|    |                                                                                                |         |
|----|------------------------------------------------------------------------------------------------|---------|
| 55 | Equivalent $\text{Na}_2\text{CO}_3$ produced by solution mining annually, tons                 | 206,000 |
|    | Same, by dry mining, tons                                                                      | 294,000 |
| 60 | Total, tons                                                                                    | 500,000 |
|    | Percent of total produced by solution mining                                                   | 41      |
|    | Percent of total produced by dry mining                                                        | 59      |
|    | Tons of water required per ton equivalent $\text{Na}_2\text{CO}_3$ produced by solution mining | 7.53    |
| 65 | G. P. M. supplied for solution mining                                                          | 711     |
|    | Time required for dry mining a panel, days                                                     | 204     |
|    | Time required for solution mining a panel, days                                                | 204     |
| 70 | Time for water to fill empty space containing the pillars, days                                | 42      |

In this example, a panel has the assumed dimensions of about 1275 feet long by 802 feet wide and contains about 449,160 tons of clear trona, not including the top approximate 3 feet of trona of a 10 foot bed, which is heavily contaminated

with shale and which is estimated as being lost, although in practice we recover a considerable amount of it by our process. Of the 449,160 tons recoverable trona estimated as being in the panel, about 52% of the total is recovered by dry mining and of the remaining 48%, a sufficient amount is recovered so that recovery by solution mining is 41% of the total production.

When the solution of trona from the pump 30, which is an approximately saturated solution at 70° F. reaches the surface, it may be heated to approximately boiling temperature and additional dry mined trona may be dissolved therein.

A boiling hot saturated solution of pure trona or sodium sesquicarbonate and water contains about 2.77 lbs. H<sub>2</sub>O per pound of equivalent Na<sub>2</sub>CO<sub>3</sub>, but the solution at 70° F. produced by solution mining contains 7.53 lbs. water per pound equivalent Na<sub>2</sub>CO<sub>3</sub>, leaving a surplus of 4.76 lbs. water which will dissolve 1.73 lbs. equivalent Na<sub>2</sub>CO<sub>3</sub>; but only 1.43 lbs. must be dissolved to correspond to the assumed production of dry mined trona, which in turn corresponds to 1 lb. equivalent Na<sub>2</sub>CO<sub>3</sub> produced by solution mining. This leaves 0.85 lb. surplus water which must be evaporated, corresponding to 2.43 lbs. total equivalent Na<sub>2</sub>CO<sub>3</sub>, or 0.34 lb. water per pound total equivalent Na<sub>2</sub>CO<sub>3</sub>. This is not a serious additional load on the evaporative system used where dry mining alone is practiced, because with dry mining alone the necessary evaporation is 2.77 lbs. per lb. equivalent Na<sub>2</sub>CO<sub>3</sub> if the dry mined trona is dissolved in boiling hot water as a step in its processing so the additional evaporative load is only about 12½%, which is of little consequence when the value of the sodium carbonate won by solution mining and brought to the surface at little additional cost is taken into consideration. The dried trona may be used as such or may be calcined to produce sodium carbonate.

While we have described a preferred method of applying our invention, it will be understood that solution mining may be carried out in one portion of the bed as described, for example, in the patent to R. D. Pike, No. 2,388,009, while dry mining is being carried out in another portion of the bed, and that the dry mined trona may be added to the solution mined trona in the manner described herein; also that various other modifications and changes may be made in the dry and solution mining operation and the recovery of the trona, and that the processes described herein may be applied to the recovery of other soluble salts, without departing from the spirit of this invention or the scope of the appended claims.

We claim:

1. A process for recovering sodium carbonate from trona beds, which comprises dry mining the trona, introducing water at substantially the temperature of the trona deposit into the dry mined sections of the bed to remove residual trona after the dry mining, bringing the solution of trona to the surface, heating said solution and dissolving in it dry mined trona, and processing to produce sodium carbonate.

2. A process for recovering sodium carbonate from trona beds, which comprises dry mining the trona bed, introducing water at a temperature not lower than ground temperature into the dry mined sections of the bed to remove residual trona after the dry mining by solution, bringing

the solution to the surface, heating said solution and dissolving dry mined trona in it and processing to produce sodium carbonate.

3. A process for recovering sodium carbonate from trona beds, comprising dry mining the trona bed, removing residual trona after dry mining by solution mining at substantially the temperature of the trona deposit, pumping the solution to the surface, heating and dissolving in it dry mined trona, and processing to produce sodium carbonate.

4. The method of recovering sodium carbonate from underground deposits of trona which comprises introducing water into the underground deposit of trona at substantially the temperature of the underground deposit, withdrawing a solution substantially saturated with trona at the underground temperature and bringing said solution above ground, heating said solution to approximately boiling temperature and dissolving more trona therein and processing said solution to produce sodium carbonate therefrom.

5. The method of mining crystallizable salts having two components of different solubilities but each having substantially greater solubility at higher temperatures than at lower temperatures which comprises introducing water into the salt deposit at substantially the temperature of said deposit contacting the deposit with the water until the water is substantially saturated by solubilizing said deposit, removing the solution from the deposit and adding heat thereto, dissolving more of said salt in said solution and recovering the salt from said solution.

6. A method for the continuous mining of the deposits of Green River trona which comprises removing about one half of the trona in a section of the mine by dry mining leaving mined out rooms with the roof supported by pillars of the unmined trona, erecting barriers isolating a portion of the mined out section remote from current dry mining operations, flooding the isolated area with water at approximately the temperature of the trona deposit, dissolving out the unmined trona with the introduced water until the introduced water is substantially saturated with trona, pumping the aqueous solution to the surface, heating the solution to approximately its boiling point, adding previously dry mined trona until the introduced trona approximates the solubilized trona, and recovering the sodium carbonate content of the heated water whereby new sections are made available for solution mining at substantially the same rate as the trona in solution mined sections is exhausted.

ROBERT D. PIKE.  
MAX Y. SEATON.

#### REFERENCES CITED

60 The following references are of record in the file of this patent:

#### UNITED STATES PATENTS

| Number    | Name    | Date          |
|-----------|---------|---------------|
| 1,121,225 | Bradley | Dec. 15, 1914 |
| 2,200,665 | Bolton  | May 14, 1940  |
| 2,388,009 | Pike    | Oct. 30, 1945 |

#### FOREIGN PATENTS

| Number     | Country | Date |
|------------|---------|------|
| 70 135,722 | Germany | 1902 |
| 198,375    | Germany | 1908 |